

[54] **PHOTOCONDUCTIVE  
1,2,3,4-TETRAHYDROQUINOLINES  
EMPLOYED IN ELECTROPHOTOGRAPHY**

[75] Inventors: **Wilhelmus Janssens, Aarschot; Johannes Josephus Vanheertum, Halle-Zandhoven; Robert Joseph Pollet, Vremde; Hendrik Hubert Sneyers, Wijnegem; Jozef Aime Dierckx, Mechelen, all of Belgium**

[73] Assignee: **Agfa-Gevaert N.V., Mortsel, Belgium**

[22] Filed: **Nov. 9, 1972**

[21] Appl. No.: **304,939**

[30] **Foreign Application Priority Data**

Nov. 10, 1971 Great Britain ..... 52287/71

[52] **U.S. Cl. .... 96/1.8, 96/1 PC, 96/1.5, 96/1.6, 96/1.7, 252/501, 260/240 E, 260/240.1**

[51] **Int. Cl. .... G03g 5/06**

[58] **Field of Search. .... 96/1.5, 1 PC, 1.8; 252/501**

[56] **References Cited**

## UNITED STATES PATENTS

3,620,742 11/1971 Willems et al. .... 96/1.5 X

|           |         |                        |          |
|-----------|---------|------------------------|----------|
| 3,684,505 | 8/1972  | Vanheertum et al. .... | 96/1.5 X |
| 3,660,084 | 5/1972  | Vanheertum et al. .... | 96/1.5 X |
| 3,307,940 | 3/1967  | Hoegl et al. ....      | 96/1.5 X |
| 3,560,209 | 2/1971  | Jenkins et al. ....    | 96/1.5 X |
| 3,232,755 | 2/1966  | Hoegl et al. ....      | 96/1.5 X |
| 3,686,153 | 8/1972  | Ono et al. ....        | 96/1.5 X |
| 3,647,428 | 3/1972  | Ono et al. ....        | 96/1.5   |
| 3,707,369 | 12/1972 | Ono et al. ....        | 96/1.5   |
| 3,730,711 | 5/1973  | Ono et al. ....        | 96/1.5   |
| 3,155,503 | 11/1964 | Cassiers et al. ....   | 96/1.5 X |
| 888,016   | 7/1971  | Just. ....             | 96/126   |

## FOREIGN PATENTS OR APPLICATIONS

|           |        |                     |        |
|-----------|--------|---------------------|--------|
| 1,245,924 | 9/1971 | Great Britain ..... | 96/1.5 |
| 1,588,977 | 4/1970 | France .....        | 96/1.5 |

*Primary Examiner*—Norman G. Torchin

*Assistant Examiner*—John R. Miller

*Attorney, Agent, or Firm*—William J. Daniel

[57] **ABSTRACT**

Electrophotographical recording process wherein a pattern of increased conductivity is produced image-wise in a photoconductive insulating recording layer containing as essential photoconductive compound a photoconductive 1,2,3,4-tetrahydroquinoline. The photoconductive compound can be chemically and spectrally sensitized and charged either negatively or positively.

40 Claims, No Drawings

1

**PHOTOCONDUCTIVE  
1,2,3,4-TETRAHYDROQUINOLINES EMPLOYED  
IN ELECTROPHOTOGRAPHY**

This invention relates to recording and reproduction of information-wise modulated electromagnetic radiation and to recording materials suitable therefor, particularly to such processes and recording materials containing one or more organic photoconductive compounds as hereinafter described.

It has now been found that a particularly photosensitive photoconductive recording member can be formed by using in its composition a photoconductive compound corresponding to the following general formula (I) :



wherein:

$Z_1$  represents the necessary atoms to close an adjacent aromatic nucleus or an adjacent aromatic ring system including an adjacent aromatic nucleus or aromatic ring system substituted with (a) non-ionic substituent(s) e.g. substituted with an alkyl group for example methyl, halogen e.g. F, Cl, Br or I, an alkoxy group e.g. methoxy, an amino group, a substituted amino group e.g. a monoalkylamino or di-alkylamino group or a cyano group,

$Z_2$  represents the necessary methylene groups or substituted methylene groups to close a 6-membered heterocyclic nitrogen-containing nucleus. Suitable substituents for the methylene groups are one or more  $C_1-C_4$  alkyl groups e.g. methyl, and

$R$  represents hydrogen, an aliphatic radical including a saturated aliphatic radical, an unsaturated aliphatic radical, a cyclo-aliphatic radical and these radicals in substituted form, or an alkylene group which is ring-closed with the carbon atom in peri-position of the aromatic ring closed by  $Z_1$  in order to form a julolidine compound.

According to a preferred embodiment  $R$  represents an organic group that can be introduced by alkylation, for example an alkyl radical including a substituted alkyl radical, e.g. methyl, a cycloalkyl radical, e.g. cyclohexyl, an allyl radical, an aralkyl radical, e.g. benzyl.

The adjacent aromatic nucleus or ring system closed by the atoms represented by  $Z_1$  is preferably one of the unsubstituted or substituted nuclei or ring systems represented by the following structural formulae:



(benzene)



(naphthalene)



(anthracene)



(carbazole)

wherein R represents hydrogen or an alkyl group e.g. methyl or ethyl



(indole)

10 15 wherein R represents hydrogen or an alkyl group, e.g. methyl or ethyl.



(dibenzofuran)  
(dibenzothiophene)

wherein : X represents oxygen or sulphur



(benzofuran)  
(benzothiophene)

wherein : X represents oxygen or sulphur



(phenothiazine)  
(phenoxazine)

wherein : X represents oxygen or sulphur, and R represents hydrogen or an alkyl group, e.g. methyl or ethyl.



(fluorine)



(indene)



(xanthene)



(quinolin-2-one)

55 60 wherein : R is hydrogen or an alkyl group, e.g. methyl or ethyl.

65 Preferred photoconductive compounds according to the present invention and which are considered as new compounds are within the scope of the following general formula (II) :



wherein :

Z<sub>1</sub> and Z<sub>2</sub> have the same significance as described in the above general formula, and A represents a bivalent organic radical of the type that can be introduced by alkylation, e.g. A represents an alkylene group, a substituted alkylene group or an alkylene chain interrupted by a bivalent aromatic group. Preferably A represents -CH<sub>2</sub>-CH<sub>2</sub>- or



Particular examples of photoconductive compounds according to the general formula (I) are listed in the following Table I.

| No.     | R <sub>2</sub>  | A                                       | X                                 | Y                 | Melting point, °C. |
|---------|-----------------|-----------------------------------------|-----------------------------------|-------------------|--------------------|
| 1.....  | CH <sub>3</sub> | (CH <sub>2</sub> ) <sub>2</sub>         | H                                 | H                 | 107                |
| 2.....  | H               | (CH <sub>2</sub> ) <sub>2</sub>         | H                                 | H                 | 151                |
| 3.....  | CH <sub>3</sub> | (CH <sub>2</sub> ) <sub>2</sub>         | 6-C <sub>2</sub> H <sub>5</sub> O | H                 | 127                |
| 4.....  | CH <sub>3</sub> | (CH <sub>2</sub> ) <sub>2</sub>         | 6-CH <sub>3</sub>                 | H                 | 179                |
| 5.....  | CH <sub>3</sub> | (CH <sub>2</sub> ) <sub>2</sub>         | 6-CH <sub>3</sub>                 | 7-CH <sub>3</sub> | 172                |
| 6.....  | H               | CH <sub>2</sub> -phenyl-CH <sub>2</sub> | H                                 | H                 | 124                |
| 10..... | CH <sub>3</sub> | CH <sub>2</sub> -phenyl-CH <sub>2</sub> | H                                 | H                 | 163                |

The preparation of the compounds according to the formula of Table I proceeds by hydrogenation of the corresponding 1,2-di-hydroquinoline compounds which are prepared e.g. according to a procedure described in the Belgian Pat. Specification Nos. 775,786 filed Nov. 25, 1971 and 776,380 filed Dec. 8, 1971 both by Agfa-Gevaert N.V.

The substitution of the hydrogen atom in the NH group of the Z<sub>2</sub>-ring by an organic group may proceed

TABLE I



| Number  | R <sub>1</sub>         | R <sub>2</sub>                                                          | X                                   | Y                                                          | Melting or boiling point             |
|---------|------------------------|-------------------------------------------------------------------------|-------------------------------------|------------------------------------------------------------|--------------------------------------|
| 1.....  | phenyl-CH <sub>2</sub> | CH <sub>3</sub>                                                         | 6-CH <sub>3</sub>                   | 7-CH <sub>3</sub>                                          | Oily product                         |
| 2.....  | H                      | CH <sub>3</sub>                                                         | 6-CH <sub>3</sub>                   | 7-CH <sub>3</sub>                                          | Oily product 105-106° C./0.5 mm. Hg. |
| 3.....  | CH <sub>3</sub>        | CH <sub>2</sub>                                                         | H                                   | H                                                          | 98-100° C./1 mm. Hg oily product.    |
| 4.....  | CH <sub>3</sub>        | H                                                                       | H                                   | H                                                          | Oily product 130-132° C./15 mm. Hg.  |
| 5.....  | phenyl-CH <sub>2</sub> | H                                                                       | H                                   | H                                                          | 145-149° C./0.2 mm. Hg.              |
| 6.....  | H                      | (1)-CH <sub>2</sub> -CH <sub>2</sub> -CH <sub>2</sub> -(8) (julolidine) | CH <sub>3</sub>                     | 6-C <sub>2</sub> H <sub>5</sub> O                          | 148-151° C./3 mm. Hg.                |
| 7.....  |                        |                                                                         | H                                   | (8)-CH <sub>2</sub> -CH <sub>2</sub> -CH <sub>2</sub> -(1) | Oily product 105-109° C./1 mm. Hg.   |
| 8.....  | phenyl-CH <sub>2</sub> | CH <sub>3</sub>                                                         | 6-C <sub>2</sub> H <sub>5</sub> -O- | H                                                          | 86° C.                               |
| 9.....  | phenyl-CH <sub>2</sub> | CH <sub>3</sub>                                                         |                                     |                                                            | 138° C.                              |
| 10..... | H                      | CH <sub>3</sub>                                                         |                                     |                                                            | 116° C.                              |

Particularly useful photoconductive compounds according to the general formula (II) are listed in the following Table II. These compounds are called "duplo compounds" for they include two 1,2,3,4-tetrahydroquinoline nuclei.

according to known alkylating techniques. This alkylation may be carried out before or after the hydrogenation of the double bond between the three- and four-carbon atom in the 1,2-dihydroquinoline compound.

For introducing an alkyl substituent by substitution of the hydrogen atom of said NH group any suitable alkylating agent e.g. trialkyl phosphate, alkyl iodides, alkyl bromides and alkyl chlorides may be used, the latter preferably in conjunction with a small amount of potassium iodide.

The preparation of the "duplo-compounds" as e.g. represented in Table II proceeds by linking together two 1,2,3,4-tetrahydro-quinolines by alkylation through the nitrogen atoms in the 1-position.

TABLE II



As suitable bifunctional alkylating agents are to be mentioned dihalogenated reactants of the formula Hal-A-Hal in which Hal represents a replaceable halogen atom e.g. chlorine, bromine or iodine and A has the same significance as described above.

The following are illustrative of reactants that may be used in the preparation of the duplo-compounds :

ethylene dichloride, dibromide and diiodide  
1-chloro-2-bromoethane  
propylene dichloride, dibromide and diiodide  
trimethylene dichloride, dibromide and bromoiodide  
butylene dichloride, dibromide and diiodide  
tetramethylene dichloride, dibromide and diiodide  
pentylene dichloride, dibromide and diiodide  
hexamethylene dichloride dibromide and diiodide  
hexylene dichloride, dibromide and diiodide  
octylene dichloride, dibromide and diiodide  
pentamethylene dichloride, dibromide and diiodide  
alpha, beta-styrene dichloride, dibromide and diiodide  
1,2-dibromocyclohexane  
1,3-dibromobutane  
1,2-dibromobutane  
1,4-dichlorobutene-2  
2-phenyl-1,2-dibromopropane  
1-p-tolyl-1,2-dichloroethane  
1,4-di(chloromethyl)benzene  
1,4-di(bromomethyl)benzene  
1,4-di(iodomethyl)benzene  
1-(2,4-dichlorophenyl)-1,2-dichloroethane  
1-(p-chlorophenyl)-1,2-dibromoethane  
decamethylene dichloride, dibromide and diiodide  
dodecamethylene dichloride, dibromide and diiodide  
1,2-dibromobutene-3  
1,2-dichloropentene-4  
1,2-dichloro-3-methylbutene-3  
1,4-dichlorobutene-2  
1,4-dibromo-2,3-dimethylbutene-2  
1,2-dichlorocyclopentene-3  
1,4-dibromocyclopentene-2  
1,4-dibromo-2,6-dimethylheptene-2  
2,3-dichloro-2,6-dimethyloctene-6

Other suitable reactants for the duplo-compound formation are the  $\beta$ -chloroethyl ester of p-tolusulphonic acid and the p-tolusulphonic acid glycol diester.

Preferred reactants are sym.-dibromoethane and sym.-dichloroethane.

The acid produced during the alkylation reaction may be neutralized by any alkaline neutralizing agent ordinarily employed for neutralizing acids produced in condensation reactions e.g. an organic base.

The following preparations illustrate in more details the manufacture of the compounds enumerated in the Tables I and II.

#### PREPARATION OF COMPOUND 5 OF TABLE I

0.1 mole of the corresponding 1,2,3,4-tetrahydroquinoline was mixed with 0.3 mole of benzyl chloride in the presence of 0.12 mole of anhydrous sodium carbonate in 150 ml of ethanol. The reaction mixture was refluxed for 6 h whereupon it was filtered. The solvent was removed from the filtrate by evaporation. The residue was washed with cold methanol and distilled under reduced pressure. The fraction boiling between 145° C and 149° C at 0.2 mm Hg was collected.

Compound 1 of Table I was prepared analogously.

Compounds 8 and 9 were recrystallized from acetone

nitrile.

#### PREPARATION OF COMPOUND 2 OF TABLE I

0.2 mole of the corresponding 1,2-dihydroquinoline and 4 ml of a dispersion of Raney nickel were mixed with 150 ml of dioxan. Hydrogen pressure of 1,500 psi was applied and the hydrogenation effected at 70° C for 2 h. The measured hydrogen acceptance corresponded with the theoretically possible value. After removal by filtering of the Raney nickel the solvent was removed by evaporation and the residue distilled under reduced pressure with the help of a fractionating column. The fraction boiling between 105°-106° C at 0.5 mm Hg was collected.

Compounds 3 and 10 of Table I were prepared analogously.

Compound 10 was not distilled but recrystallized from ligroin in the presence of active carbon.

#### PREPARATION OF COMPOUND 4 OF TABLE I

A mixture of 0.2 mole of 1,2,3,4-tetrahydroquinoline, 0.4 mole of trimethyl phosphate and 0.21 mole of ethyl diisopropylamine were heated at 140° C on an oil-nath for 1 h.

The reaction mixture was poured into water and treated with sufficient ammonium hydroxide for obtaining a slightly alkaline reaction.

The obtained supernatent oily product was extracted with chloroform. The whole mixture was washed with 2N aqueous hydrochloric acid and thereupon washed with water until neutral. After drying on anhydrous sodium sulphate the extract was distilled under reduced pressure with a distillation column and the fraction boiling between 130°-132° C at 15 mm Hg collected.

#### PREPARATION OF COMPOUND 6 OF TABLE I

90.5 g of the corresponding 1,2-dihydroquinoline were hydrogenated in the presence of Raney nickel under 1,500 psi of hydrogen pressure at 70° C in dioxan as a solvent. After removal of the Raney nickel by filtering the solvent was evaporated under reduced pressure and the hydrogenated product purified by distillation. The fraction boiling between 148°-151° C at 3 mm Hg was collected.

#### PREPARATION OF COMPOUNDS 1, 3, 4 and 5 OF TABLE II

The hydrogenation of the corresponding 1,2-dihydroquinoline to the indicated 1,2,3,4-tetrahydroquinoline of Table II proceeded in a total liquid volume of 300 ml by using 0.1 mole of the 1,2-dihydroquinoline, 3 ml of Raney nickel dispersion and the balance of dioxan at 1,500 psi. The hydrogenation was effected at 85° C for 2 h. The hydrogen acceptance was slightly more than the theoretical value. After removal of the Raney nickel by filtering the solvent was evaporated.

Compound 1 was recrystallized from acetonitrile, compound 3 from butanol and compounds 4 and 5 from ethanol.

#### PREPARATION OF COMPOUND 2 OF TABLE II

The alkylation was carried out by heating with stirring 0.2 mole of the 1,2,3,4-tetrahydroquinoline with 0.1 mole of sym.-dibromoethane and 0.2 mole of triisopropanolamine at 100° C for 10 h. The obtained reac-

tion product was extracted with dichloroethane and washed first with 2N aqueous hydrogen chloride and then with water until neutral.

The extract was dried over anhydrous sodium sulphate and after filtering the solvent was removed. Recrystallization of the crude product from ethylene glycol monomethyl ether yielded a white powder.

Melting point : 151° C. Yield : 54 percent.

In the preparation of the compounds 6 and 7 of Table II 1,4-di(monochloromethyl)benzene was used instead of sym.-dibromoethane.

The photoconductive duplo compounds of Table II are particularly interesting for their high photosensitivity and pure state wherein they can be separated. Most of these products are obtained as white powders, which are suited for producing very clear colourless photosensitive layers.

The photoconductive compounds applied according to the present invention may be used alone or in combination with substances imparting desired chemical or physical properties to the recording element. So, these substances may be combined with other substances that either or not are photoconductive and exert an influence e.g. on the dark-resistivity, the dischargeability of conductivity of the recording layer by an exposure to electromagnetic radiation, or on the transparency or the quality of the final image, e.g. by counteracting the fringe effect as described in the United Kingdom Pat. specification No. 1,007,349 filed Oct. 12, 1961 by Gevaert Photo-Producten N.V.

A proper combination with selected binding agents and/or chemical sensitizing agents may result in an enhancement of the total sensitivity. The recording elements according to the present invention preferably contain at least 5 percent by weight of a photoconductive 1,2,3,4-tetrahydroquinoline derivative being within the scope of the above general formulae. For use in electrophotography the recording element preferably consists for at least 10 percent by weight of one or more of the said 1,2,3,4-tetrahydroquinoline derivatives. The electrically insulating binding agent used in a recording layer containing said derivative may provide the desired mechanical strength for instance to form a self-supporting layer, and preferably has a resis-

tivity of at least 10<sup>9</sup> ohm.cm.

According to a particular embodiment the recording layer consists of the photoconductor, which, e.g., has been applied to a suitable support in molten state forming a micro-crystalline or glass-like layer on cooling. This technique can be applied when the photoconductive recording element has not to possess a high mechanical strength. For such technique reference is made to the Canadian Pat. specification No. 712,541 filed Feb. 5, 1960 by Gevaert Photo-Producten N.V.

Macromolecular compounds suitable for use as insulating binding agent for the photo-conductive compounds are, e.g., natural resins such as dammar resin, gum arabic, microcrystalline waxes, modified natural substances such as cellulose diacetate, cellulose triacetate, and ethylcellulose, pentaerythrite polyesters or modified colophony resins and ester gums, polymers such as polyethylene, polystyrene and copolymers of styrene, polyvinyl acetate and copolymers of vinyl acetate, polyvinyl acetals of formaldehyde, acetaldehyde or butyraldehyde, polyacrylic acid esters and polymethacrylic acid esters, coumarine-indene resins, epoxy resins and polycondensates such as glycerolphthalate resins and other glyceryl polyesters, alkyd resins, diethylene glycol polyesters, formaldehyde resins and silicone resins.

Preferred binding agents are halogen-containing polymers and epoxy resins combined with silicone resins. The sensitization of organic photoconductors with halogen-containing polymers is described in the United Kingdom Pat. specification No. 964,878 filed May 3, 1960 by Gevaert Photo-Producten N.V. According to said specification a material suitable for use in electrophotography comprises a photoconductive layer incorporating an organic monomeric photoconductor and a halogen-containing polymer in such layer or in a juxtaposed layer (if any), the sensitivity of said photoconductor having been increased by making it to interact with said halogen-containing polymer by heating.

In the following Table III a list of preferred polymeric binding agents is given, which may be used in combination with the heterocyclic organic photoconductors of use according to the present invention as well as the corresponding suitable solvents.

TABLE III

Polymeric binding agent defined by its structural unit(s)

Solvent

Methylene chloride.



Do.



Do.



Do.



Do.

Table III—Continued

| Polymeric binding agent defined by its structural unit(s) | Solvent                           |
|-----------------------------------------------------------|-----------------------------------|
|                                                           | Do.                               |
|                                                           | Do.                               |
|                                                           | Do.                               |
|                                                           | Do.                               |
|                                                           | Do.                               |
|                                                           | Do.                               |
| 25% by weight                                             |                                   |
|                                                           | Do.                               |
|                                                           | Do.                               |
|                                                           | Do.                               |
|                                                           | Do.                               |
| 10% by weight                                             |                                   |
| 80% by weight                                             |                                   |
| 10% by weight                                             |                                   |
|                                                           | Methylene chloride/acetone (1:1). |
| 91% by weight                                             |                                   |
| 3% by weight                                              |                                   |
| 6% by weight                                              |                                   |

Table III—Continued

| Polymeric binding agent defined by its structural unit(s)                                                                                                              | Solvent                                            |
|------------------------------------------------------------------------------------------------------------------------------------------------------------------------|----------------------------------------------------|
| <br> | Do.<br>Methylene chloride/acetone/ethanol (1:1:1). |

According to a special embodiment the photoconductive compounds applied according to the present invention are used in admixture with inorganic and organic photoconductive substances known to those skilled in the art, e.g. sulphur, selenium, photoconductive oxides, sulphides, and selenides of zinc, cadmium, mercury, antimony, bismuth, lead, anthracene, anthraquinone, and photoconductive polymers e.g. those containing N-vinylcarbazole recurring units and other known monomeric and polymeric organic photoconductors, e.g. those described in the published Dutch Pat. application No. 70/04174 filed Mar. 24, 1970 by Gevaert-Agfa N.V.

The inherent spectral sensitivity of most of the photoconductive compounds listed in Tables I and II is mainly situated in the near U.V. range, i.e., in the range of 360 to 420 nm.

The spectral sensitivity of recording materials according to the present invention can be increased in different ways, e.g. by adding so-called spectral sensitizing agents for the photoconductive substances contained in the recording element or by admixing to the said heterocyclic organic photoconductive compounds other photoconductive substances, whose inherent sensitivity for a particular part of the electromagnetic radiation spectrum is higher than that of the present compounds.

Suitable spectral sensitizing dyestuffs for the organic photoconductor are among others organic dyestuffs, known as methine dyes, or xanthene dyes of which the phthaleins and rhodamines are subclasses, and triaryl-methane dyes e.g. crystal violet (C.I. 42,555) and the triarylmethane dyes described in published Dutch Pat. application No. 6,704,706 filed April 3, 1967 by Gevaert-Agfa N.V. The term methine dyes includes mono- as well as polymethine dyes, which dyes are known to those skilled in the art of the spectral sensitization of light-sensitive silver halide. Preferred methine dyes are 55 of the cationic type. As preferred xanthene dyes Rhodamine B (C.I. 45,170), Rose Bengal (C.I. 45,440) and Fluorescein (C.I. 45,350) are mentioned. The spectral sensitizing dyes are preferably added to the recording layer composition in a proportion of 0.01 to 5 percent by weight in respect of the photoconductive substance(s).

Particularly preferred methine dyes are within the scope of the following general formulae :

1.



65

wherein :

$A_1$  stands for a dimethine or tetramethine group including a substituted dimethine or tetramethine group,

$n$  stands for one or two,

$R_1$  stands for alkyl including substituted alkyl, an unsaturated aliphatic group e.g. allyl, aralkyl including substituted aralkyl, aryl including substituted aryl or cycloalkyl,

$R_2$  stands for alkyl, aryl including substituted aryl, e.g. phenyl and phenyl substituted preferably in the *p*-position by alkyl, halogen and alkoxy, a 5- or 6-membered heterocycle whose heteroatom is oxygen, sulphur, selenium or nitrogen such as 2-, 3-, or 4-pyridyl, 2-furyl, 2-thienyl, etc. including their quaternary salts,

$R_3$  stands for hydrogen or has one of the significances given for  $R_1$ ,

$R_4$  stands for hydrogen, alkyl, alkoxy or halogen or together with  $R_3$  forms an alkylene bridge such as dimethylene and trimethylene,

each of  $R_5$  and  $R_6$  (the same or different) stands for hydrogen, alkyl, alkoxy or halogen or together represent the atoms necessary to complete a fused-on benzene nucleus,

$X_1^-$  represents an anion e.g.  $Cl^-$ ,  $Br^-$ ,  $I^-$ ,  $ClO_4^-$ ,  $CH_3SO_4^-$ , or



but is missing when the  $R_1$  group contains already an anion (betaine type salt), and

$Z$  represents the atoms necessary to complete a heterocyclic nucleus of the types used in the production of cyanine dyes e.g. such as those of the thiazole series, e.g. thiazole, 4-methylthiazole, 4-methyl-5-carbethoxythiazole, 4-phenylthiazole, 5-methylthiazole, 5-phenylthiazole, 4-(*p*-tolyl)-thiazole, 4-(*p*-bromophenyl)-thiazole, 4,5-dimethylthiazole, 4,5-diphenylthiazole, 4-(2-thienyl)-thiazole, 4-(*m*-nitrophenyl)-thiazole, those of the benzothiazole series, e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 6-sulphobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, 4,5,6,7-tetrahydrobenzo-

thiazole, 5,6-dimethoxybenzothiazole, 5,6-dioxymethylenebenzothiazole, 5-hydroxybenzothiazole, 6-hydroxybenzothiazole, 5,6-dimethylbenzothiazole, those of the naphthothiazole series e.g. naphtho[2,1-*d*]thiazole, naphtho[1,2-*d*]thiazole, 5-methoxynaphtho[1,2-*d*]thiazole, 5-ethoxynaphtho[1,2-*d*]thiazole, 3-methoxynaphtho[2,1-*d*]thiazole, 7 methoxynaphtho[2,1-*d*]thiazole, those of the thionaphtheno[7,6-*d*]thiazole series e.g. 7-methoxythionaphtheno[7,6-*d*]thiazole, those of the thiadiazole series e.g. 4-phenylthiadiazole, those of the oxazole series e.g. 4-methyloxazole, 5-methyloxazole, 4-phenyloxazole, 4,5-diphenyloxazole, 4-ethyloxazole, 4,5-dimethyloxazole, 5-phenyloxazole, those of the benzoxazole series e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole, those of the naphthoxazole series, e.g. naphtho[2,1-*d*]oxazole, naphtho[1,2-*d*]oxazole, those of the selenazole series e.g. 4-methylselenazole, 4-phenylselenazole, those of the benzoselenazole series e.g. benzoselenazole, 5-chlorobenzoselenazole, 5-methoxybenzoselenazole, 5-methyl-6-methoxybenzoselenazole, 5,6-dioxymethylenebenzoselenazole, 5-hydroxybenzoselenazole, 4,5,6,7-tetrahydrobenzoselenazole, those of the naphthoselenazole series e.g. naphtho[2,1-*d*]selenazole, naphtho[2,1-*d*]selenazole, those of the thiazoline series e.g. thiazoline, 4-methylthiazoline, 4-hydroxymethyl-4-methylthiazoline, 4,6-bis-hydroxymethylthiazoline, those of the oxazoline series e.g. oxazoline, those of the selenazoline series e.g. selenazoline, those of the 2-quinoline series e.g. quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc., those of the 4-quinoline series e.g. quinoline, 6-methoxyquinoline, 7-methylquinoline, 8-methylquinoline, those of the 1-isoquinoline series e.g. 1-isoquinoline, 3,4-dihydroisoquinoline, those of the 3-isoquinoline series e.g. 3-isoquinoline, those of the pyrimidine series, those of the quinoxaline series, those of the quinazoline series, those of the 1phthalazine series, those of the 2-pyridine series, e.g. pyridine, 5-methylpyridine, 3-nitropyridine, those of the 3,3-dialkylindolenine series, e.g. 3,3-dimethylindolenine, 3,3,5-trimethylindolenine, 3,3,7-trimethylindolenine, etc., those of the benzimidazole series e.g. benzimidazole, 5,6-dichlorobenzimidazole, 5-chlorobenzimidazole, 5,6-dibromobenzimidazole, 5-chloro-6-amino-benzimidazole, 5-chloro-6-bromobenzimidazole, 5-phenylbenzimidazole, 5-fluorobenzimidazole, 5,6-difluorobenzimidazole, 5-cyanobenzimidazole, 5,6-dicyanobenzimidazole, 5-chloro-6-cyanobenzimidazole, 5-fluoro-6-cyanobenzimidazole, 5-acetylbenzimidazole, 5-chloro-6-fluorobenzimidazole, 5-carboxybenzimidazole, 7-carboxybenzimidazole,

5-carbethoxybenzimidazole, 7-carbethoxybenzimidazole, 5-sulphamylbenzimidazole, or 5-N-ethylsulphamylbenzimidazole, 5-ethylsulphonylbenzimidazole and 5-trifluoromethylsulphonylbenzimidazole;



wherein :

A<sub>2</sub> stands for a monomethine or trimethine group including a substituted monomethine or trimethine group,  
each of R'<sub>2</sub> - R'<sub>6</sub> and R''<sub>2</sub> - R''<sub>6</sub> (the same or different) has one of the significances given for R<sub>2</sub> - R<sub>6</sub>,  
X<sub>2</sub><sup>-</sup> has the same significance as X<sub>1</sub><sup>-</sup>;



25 wherein :

each of R'<sub>1</sub> and R''<sub>1</sub> (the same or different) has one of the meanings given for R<sub>1</sub>,  
X<sub>3</sub><sup>-</sup> has the same meaning as X<sub>1</sub><sup>-</sup>,  
A<sub>3</sub> has the same meaning as A<sub>2</sub>,  
each of m and p (the same or different) stands for one or two, and  
each of Z<sub>1</sub> and Z<sub>2</sub> (the same or different) stands for the atoms necessary to complete a heterocyclic nucleus of the thiazole, benzothiazole, naphthothiazole, thionaphtheno[7,6-*d*]thiazole, thiadiazole, oxazole, benzoxazole, naphthoxazole, selenazole, benzoselenazole, naphthoselenazole, 2-quinoline, 4-quinoline, pyrimidine, quinoxaline, quinazoline, 2-pyridine, 3,3-dialkylindolenine or of the benzimidazole series;  
representative examples of these heterocyclic nuclei can be found above in the definition of Z in formula I.

40 45 The dyestuffs corresponding to the above general formulae can be prepared according to the methods known by those skilled in the art of methine dye chemistry.

50 According to a further embodiment of the invention the recording material contains one or more substances that increase the photoconductivity of the recording material in the inherent spectral sensitivity range of the said heterocyclic organic photoconductive compounds. As already has been said a binding agent can act as a sensitizing agent that enhances the total sensitivity of the recording element. In that respect are to be mentioned compounds containing one or more electron-attracting atoms or groups, e.g. those that are known as non-ionic Lewis acids, e.g. the Lewis acids that can form a "charge transfer complex" as described e.g. in the U.S. Pat. specification No. 3,408,183 of Joseph Mammino issued Oct. 29, 1968. Good sensitizing results are obtained with organic carboxylic acid anhydrides and with quinones containing electron-attracting substituents, e.g. halogen or cyano, such as in tetrachlorobenzoquinone and tetracyanobenzoquinone, with organic compounds containing a



group and with the compounds according to the structural formula of the Belgian Pat. specification No. 734,141 filed June 6, 1969 by Gevaert-Agfa N.V. and the chlorine- and/or cyano-containing polymers of Table III.

The 1,2,3,4-tetrahydroquinoline derivatives may be used in admixture with diazonium salts that on exposure to electromagnetic radiation produce (a) radical(s), which irreversibly increase(s) the electroconductivity of a recording layer. Such substances as well as details about their incorporation into a recording layer containing an organic photoconductive insulating substance are described in the United Kingdom Pat. specification No. 964,872 filed Apr. 22, 1959 by Gevaert Photo-Producten N.V. and the U.S. Pat. specification No. 3,113,022 of Paul Maria Cassiers, Jean Marie Nys, Jozef Frans Willems and Rene Maurice Hart issued Dec. 3, 1963. A particularly suitable conductivity-increasing diazonium compound is p-nitrobenzene-diazonium chloride. The diazonium compounds are preferably used in an amount of 0.01 to 10 percent by weight in respect of the present photoconductive heterocyclic organic compounds.

Other additives well known in the art of preparing photoconductive coatings for recording purposes may be used, e.g. matting agents, fluorescing compounds, phosphors, optical brightening agents, agents controlling the adhesive power of the recording layer, agents controlling the elasticity, the plasticity and the hardness of the recording layer, agents controlling the viscosity of the coating composition, antioxidants, gloss-improving agents, etc.

Transparent and semi-transparent recording materials containing the photoconductive heterocyclic organic compounds as described hereinbefore are especially suited for use in recording materials applied for the production and reproduction of microfilm images. Microfilm images can be copied in contact or enlarged optically on recording materials according to the present invention. According to the type of development, the transparencies obtained (contact copies and enlargements) can serve as negative or positive intermediate prints for further printing, e.g. on diazotype materials.

The semitransparent recording materials according to the present invention preferably have an optical density not larger than 0.30 towards visible light or the copying light used in the printing apparatus wherein it is used as intermediate print.

The photoconductive heterocyclic organic compounds described hereinbefore are further especially suited for being applied in the manufacture of pigment images wherein the pigments may have the properties of a fluorescent compound or phosphor.

As is generally known luminescent phosphors are used in screens of cathode-ray tubes and more particularly in television, X-ray, radar and oscilloscope screens. It is further known that in colour television screens phosphors of different colour have to be fixed on a screen in a particular pattern.

The described photoconductive compounds are successfully used in a process for the production of colour television screens as described in the French Pat. speci-

ification No. 1,336,499 filed Sept. 26, 1962 by Comp.-Francaise Thomson-Houston. According to the process described in said specification a pattern of a phosphor on a screen support is produced by the steps of apply-

5 ing to said support a coating of an electroconductive material and to said coating a layer comprising a vapourisable or thermolysable photoconductive compound optionally incorporated in a vaporisable or thermolysable binding agent. On said coating an electrostatic 10 charge pattern corresponding with the pigment pattern to be produced is formed in an electrophotographic way, and the electrostatic charge pattern is developed with non-volatile powder particles that have the desired phosphorescent or luminescent properties. Subse- 15 quently the photoconductive layer containing the phosphor powder image is heated in order to remove the volatile substances of the photoconductive recording layer and to make the phosphor pattern adhere to the screen support.

20 In order to fix the powder image before applying the heating step it is preferably overcoated with a layer of a thermolysable binding agent.

According to said French Patent Specification photo-conductors of the group of anthracene, anthraquinone and xanthene are used. The recording layer may further contain boric acid.

The photoconductors mentioned in the French Pat. specification are advantageously partly or wholly substituted by the photoconductive substances applied according to the present invention.

Suitable thermolysable binding agents belong to the class of the polyacrylic acid esters and polymethacrylic acid esters, e.g. polymethyl methacrylate, polyethyl methacrylate and polyethyl acrylate.

35 The thickness of the photoconductive layers of the present invention is not critical but is open to choice within a wide range according to requirements in each individual case. Good results are attained with photoconductive layers of a thickness between 1 and 30  $\mu$  40 preferably between 3 and 20  $\mu$ . Too thin layers do not have a sufficient insulating power in the absence of active electromagnetic radiation, whereas too thick layers require extensive exposure times. The photoconductor may be used in a self-supporting or supported layer.

45 In the manufacture of electrophotographic recording materials according to the present invention preferably a relatively conductive support for the recording layer is used, e.g. an electroconductive sheet or plate, or an 50 insulating sheet or plate covered with an electro-conductive interlayer. By electro-conductive plate or sheet is understood a plate or sheet whose electrical resistivity is smaller than that of the non-irradiated (dark-adapted) photoconductive layer, i.e., in general smaller 55 than  $10^9$  ohm.cm and preferably is at least 100 times as small as that of the recording layer. Supports whose resistivity is not higher than  $10^7$  ohm.cm are preferred. The recording layers themselves have preferably an 60 electrical insulating power as high as possible without affecting too much the photosensitivity by means of too high an amount of insulating binding agent. Preferably the recording layers have in non-irradiated state (dark-adapted state) a resistivity of at least  $10^9$  ohm.cm.

Suitable conductive plates are, e.g., plates of metals such as aluminium, zinc, copper, tin, iron, or lead.

Suitable electro-conductive interlayers for insulating supports are, e.g., vacuum-coated metal and conduc-

tive metal compound (metal oxide or metal salt) layers such as silver, tin, aluminium, titanium dioxide and copper iodide conductive layers, transparent conductive polymer layers, e.g. applied from polymers containing quaternized nitrogen atoms, such as those described in the United Kingdom Pat. specification No. 950,960 filed Sept. 23, 1960 by Gevaert Photo-Producten N.V., or layers containing conductive particles, e.g. carbon black and metal particles dispersed in a binder. The binder used for said particles has a resistivity preferably lower than  $10^6$  ohm.cm. A suitable binder for that purpose is gelatin.

It is possible to produce transparent photoconductive recording materials by applying the photoconductive compounds together with a suitable binder (if necessary) from a clear solution to a conductive transparent base or a transparent insulating base coated with an electroconductive transparent interlayer.

As transparent bases resin sheets having an optical density of not more than 0.10 are preferred, e.g., a sheet made of polyethylene terephthalate or cellulose triacetate. The conductive interlayer preferably consists of a metal coating, e.g., a vacuum-coated aluminium layer having an optical density of not more than 0.30, or of a conductive transparent polymer layer composed, e.g., of an organic polyionic polymer, e.g. a polymer containing quaternized nitrogen atoms such as a quaternized polyethylene-imine.

In reproduction techniques wherein the prints are to be produced on an opaque background preferably a paper sheet is used as support for the recording layer.

Paper sheets that have an insufficient electrical conductivity are coated or impregnated with substances enhancing their conductivity, e.g. by means of a conductive overcoat such as a metal sheet laminated thereto.

As substances suited for enhancing the conductivity of a paper sheet and which can be applied in the paper mass are particularly mentioned hygroscopic compounds and antistatic agents as described, e.g., in the United Kingdom Pat. specification No. 964,877 filed May 2, 1960 by Gevaert Photo-Producten N.V., and antistatic agents of polyionic type, e.g. CALGON CONDUCTIVE POLYMER 261 (trade mark of Calgon Corporation, Inc. Pittsburgh, Pa., U.S.A.) for a solution containing 39.1 percent by weight of active conductive solids, which contain a conductive polymer having recurring units of the following type :



Paper sheets are preferably impermeabilized to organic solvents, e.g. by means of a water-soluble colloid or by strongly hydrating the cellulose fibers such as in the case of glassine paper.

In order to prepare an electrophotographic material according to the present invention various techniques may be applied.

In practice, the photoconductive substances involved, either alone or together with other additives such as those described above, preferably are first dissolved or dispersed in a suitable organic solvent such as

a chlorinated hydrocarbon, e.g. methylene chloride. The solution or dispersion thus obtained is uniformly spread on a surface of a suitable support, e.g. by centrifuging, spraying, brushing, or coating. Thereupon the layer formed is dried in such a way that a solid photoconductive layer is formed on the surface of the support.

Recording materials according to the present invention can be used in any of the different techniques known in recording with the aid of photoconductors. According to a preferred embodiment they are used in a technique based on the discharge of an electrostatically charged recording layer by exposure to light.

Photoconductive recording materials prepared according to the present invention can be used in exposure units equipped with incandescent lamps, so that they need not be exposed with light rays rich in ultraviolet such as those emitted by a high-pressure mercury vapour bulb.

20 The electrostatic charging of photoconductive recording elements according to the present invention can be effected according to any method known in electrophotography, e.g. by friction with a smooth material, with a material possessing a high electric resistance, e.g. a cylinder coated with polystyrene, by corona discharge, by contact charge, or by discharge of a capacitor.

Recording materials containing the said organic photoconductive substances can be used in a recording 30 technique comprising a negative corona charging as well as in a recording technique comprising a positive corona charging.

In order to obtain an electrostatic image it is possible to effect the charging and exposure steps simultaneously and even to expose the recording layer image-wise before charging since a conductivity image is formed that is not destroyed immediately, especially if diazonium salts are used in the recording element. It is preferred, however, that the charging is effected before image-wise exposure.

The electrostatic latent image can be converted into a visible image either on the electrophotographic material wherein the latent image was formed, or on a material to which the electrostatic latent image was transferred, e.g. by application of the method described in the Belgian Pat. specification No. 529,234 filed May 29, 1954 by Chester Floyd Carlson.

The conversion of the original or transferred latent image into a visible image can occur according to one of the techniques known in electrophotography, wherein use is made of a conductivity pattern (e.g. electrolysis) or the electrostatic attraction or repulsion of finely divided coloured substances, which, e.g., are present in a powder mixture, in an electrically insulating liquid (e.g. in the form of a suspension) or in a gas (e.g. in the form of an aerosol), or wherein electrostatic attraction is used for selectively wetting charged portions of the recording layer, as described in the United Kingdom Pat. specification Nos. 1,020,505 filed Nov. 8, 1961 and 1,033,419 filed Nov. 26, 1962 both by Gevaert Photo-Producten N.V.

When the sign of the charge of the developing powder or developing liquid is properly chosen, either a negative or a positive print can be obtained from any original. If both printing material and developing powder or developing liquid have the same sign of charge, the powder only adheres to the discharged areas so that

a negative print is obtained. If the signs of the recording material and of the developing powder or developing liquid differ, a positive print is obtained.

If a coloured powder is used for making visible the latent image, the visible image obtained can, if necessary, be fixed according to one of the methods known in electrophotography, e.g., by heating, or it can be transferred to another support, e.g. according to the method described in the United Kingdom Pat. specification No. 658,699 filed Apr. 14, 1949 by Battelle Memorial Institute and fixed thereon.

The present heterocyclic organic photoconductive compounds can also be supplied in a thermoplastic recording process to form a ripple-image as described, e.g., in the United Kingdom Pat. specification No. 964,881 filed May 17, 1960 by Gevaert Photo-Producten N.V.

Evidently the present invention by no means is limited to one or other particular embodiment of using the electrophotographic material containing the photoconductive compounds as described herein. The exposure technique, the charging method, the formation of the charge pattern, the transfer of such pattern if applied, the developing method, and the fixation or the transfer of the developing material pattern may be modified or adapted.

The composition of the recording materials used in these methods may be adapted to the requirements of the recording process used.

Electrophotographic materials according to the present invention can be employed in reproduction techniques, wherein different kinds of electromagnetic radiations are used, e.g. visible light, U.V.-radiation, X-rays and  $\gamma$ -rays.

The following examples illustrate the present invention.

The percentages and ratios are by weight unless otherwise indicated.

#### EXAMPLE 1

An aluminium-laminated paper sheet was coated with the following composition:

|                                                                                                    |        |
|----------------------------------------------------------------------------------------------------|--------|
| 10 % by weight solution in methylene chloride of an organic photoconductor listed in Table I or II | 50 ml. |
| copoly(vinyl chloride/vinyl acetate/maleic anhydride) (mol ratio 86.5/13.3/0.2)                    | 5 g    |
| 1,2-dichloro-ethane                                                                                | 45 ml. |

The coating was carried out in such a ratio that the dried photoconductive layer contained 2 g of photoconductor per sq.m.

After a negative corona charging with a potential difference of -6,000 V between the corona wires and the ground, the charged recording layer was contact-exposed for 30 sec through a step wedge having 0.20 log exposure increments. In this exposure 5 Osram (trade name) L 20 fluorescent tubes, mainly emitting in the U.V. range and the shorter wavelengths of the visible spectrum were placed at a distance of 20 cm from the recording layer.

The latent wedge image obtained was electrophoretically developed by means of an electrophoretic developer prepared by diluting the concentrated developer composition described hereinafter in a volume ratio of 15/1,000 by means of ISOPAR H (an isoparaffinic hydrocarbon mixture having a boiling range of 177°-188° C sold by Esso Belgium N.V., Antwerp, Belgium):

|                                                  |         |
|--------------------------------------------------|---------|
| carbon black (average particle size: 20 nm)      | 30 g    |
| zinc monotridecyl phosphate as dispersing agent  | 1.5 g   |
| ISOPAR H (trade name)                            | 750 ml. |
| resin solution prepared as described hereinafter | 150 g   |

5 The resin binder solution was prepared by heating 500 g of ALKYDAL L 67 (of Farbenfabriken Bayer A.G., Leverkusen, W.Germany for a linseed oil-modified (67 percent by weight) alkyd resin) and 500 ml of white spirit containing 11 percent by weight of aromatic compounds at 60° C till a clear solution was obtained, and subsequent cooling.

A black positive copy of the wedge original on a transparent base was obtained.

15 From the wedge prints obtained the relative speed values of the developed materials were calculated based on a comparison of the number of non-toned (discharged) steps present in the wedge prints obtained with material containing a photoconductor of Table I or II with the number of non-toned steps produced in a material containing photoconductor number 3 of Table II to which is given arbitrarily the speed value 100.

| Number of compound of Table I or II | Relative Speed values |
|-------------------------------------|-----------------------|
| 1.I                                 | 25                    |
| 2.I                                 | 2.5                   |
| 1.II                                | 250                   |
| 2.II                                | 250                   |
| 3.II                                | 100                   |
| 5.II                                | 160                   |
| 6.II                                | 160                   |
| 7.II                                | 60                    |

#### EXAMPLE 2

An electrophotographic recording material was prepared by coating onto an aluminium laminated paper a solution containing:

|                                                                                                   |         |
|---------------------------------------------------------------------------------------------------|---------|
| 10% by weight solution in methylene chloride of an organic photoconductor listed in Table I or II | 50 ml.  |
| copoly(vinyl chloride/vinyl acetate/maleic anhydride) (mol ratio 86.5/13.3/0.2)                   | 5 g     |
| Rhodamine B (C.I. Basic Violet 10 C.I. 45.170)                                                    | 0.025 g |
| 1,2-dichloroethane                                                                                | 45 ml.  |

45 The dried recording layer contained 2 g of photoconductor per sq.m.

The coated samples were negatively charged with a negative corona having a potential difference of -6,000 V between the corona wires and the ground.

50 The charged recording layer was contact-exposed for 6 sec. through a step-wedge having 0.20 log exposure increments. In the exposure tungsten filament lamp light was used.

The latent wedge images were electrophoretically developed as described in Example 1.

55 The relative speed values of the developed materials were compared with the electrophotographic material containing photoconductor number 3 of Table II which is given arbitrarily the speed value 100.

| Number of compound of Table I or II | Relative Speed values |
|-------------------------------------|-----------------------|
| 1.I                                 | 25                    |
| 2.I                                 | 1                     |
| 3.I                                 | 25                    |
| 4.I                                 | 1                     |
| 6.I                                 | 2.5                   |
| 1.II                                | 100                   |
| 2.II                                | 40                    |
| 3.II                                | 100                   |
| 5.II                                | 250                   |
| 6.II                                | 100                   |
| 7.II                                | 40                    |

## EXAMPLE 3

To a polyethylene terephthalate support of  $100 \mu$  a conductive transparent coating was applied from an aqueous solution of gelatin and CALGON CONDUCTIVE POLYMER 261 in a weight ratio of 2:1. Coating was carried out in such a way that the dried coating contained 2 g of gelatin per sq.m. The electric resistivity of the coating was  $1 \times 10^6$  ohm per sq.cm.

An electrophotographic recording material was prepared by coating onto said conductive layer a solution consisting of

methylene chloride  
1,2-dichloro-ethane



45 ml.  
45 ml.

copoly (vinyl chloride/vinyl acetate/maleic anhydride)(molar ratio 86.5/13.3/0.2)  
Rhodamine B (C.I. Basic Violet 10; C.I. 45.170)

5 g  
5 g  
0.025 g

The dried recording layer containing approximately 3 g of photoconductor per sq.m., was charged with a negative corona and contact-exposed with 100 lux.sec with the same light source as in Example 2. The latent image was electrophoretically developed for 5 sec. with the developer described in Example 1. A good copy of the original was obtained.

## EXAMPLE 4

To a polyethylene terephthalate support of  $63 \mu$  a 35 conductive transparent coating was applied from

a 10 % aqueous solution of polystyrene sulphonic acid sodium salt  
methanol

40 ml.  
60 ml.

The coating was carried out in such a way that the dried material contained 1.75 g of polystyrene sulphonic acid sodium salt per sq.m. The electrical resistivity was  $5 \times 10^6$  /cm<sup>2</sup>.

An electrophotographic recording material was prepared by coating onto said conductive layer at a coverage of 3 g per sq.m of photoconductor a solution containing :



5

5 g

copoly(vinyl chloride/vinyl acetate/maleic anhydride)(molar ratio 86.5/13.3/0.2)

5 g

methylene chloride

45 g

1,2-dichloroethane

45 g

10

15

20

25

30

35

After a negative corona charging with a potential difference of -6,000 V, the charged recording layer was contact-exposed for 30 sec through a positive transparency of a test chart with 5 Osram (trade name) L 20 fluorescent tubes at a distance of 20 cm from the recording layer.

After the exposure the latent image was developed for 5 sec with a triboelectrically charged positive toner on the base of three parts by weight of pitch, four parts by weight of colophony and three parts by weight of carbon black.

A contrasty transparent positive copy of the transparency was obtained.

## EXAMPLE 5

The effect on the speed of electrophotographic recording materials resulting from a few chemical sensitizers was examined.

Therefor the following photoconductive compositions were coated on an aluminium laminated paper:

10 % by weight solution in methylene chloride  
of the organic photoconductor number 2 of

Table II

50 ml.

40 copoly(vinyl chloride/vinyl acetate/maleic anhydride)(molar ratio 86.5/13.3/0.2)

5 g

a chemical sensitizer listed in Table IV

0.05 g

The dried layers contained 2 g of photoconductor per 45 sq.m.

Processing of the materials was carried out in the same way as described in Example 1. The relative speed values are listed hereinafter.

TABLE IV

| Test No. | Structural formula chemical sensitizer | Relative speed value |
|----------|----------------------------------------|----------------------|
| 0.....   | None.....                              | 100                  |
| 1.....   |                                        | 250                  |
| 2.....   |                                        | 250                  |

Table IV—Continued

| Test No. | Structural formula chemical sensitizer | Relative speed value |
|----------|----------------------------------------|----------------------|
| 3        |                                        | 250                  |
| 4        |                                        | 160                  |
| 5        |                                        | 400                  |
| 6        |                                        | 160                  |
| 7        |                                        | 160                  |
| 8        |                                        | 400                  |
| 9        |                                        | 250                  |
| 10       |                                        | 250                  |
| 11       |                                        | 1,600                |

## EXAMPLE 6

Electrophotographic recording materials were prepared by coating onto a conductive layer as described in Example 3 a composition containing:

compound number 4 of Table II  
copoly(vinyl chloride/vinyl acetate/maleic anhydride) (molar ratio 86.5/13.3/0.2)  
methylene chloride  
1,2-dichloroethane  
a sensitizing dye as listed in the table V

5 g 60  
5g  
45 ml  
45 ml  
0.025 g

The recording layers were charged, exposed and developed as described in Example 3.

From the obtained prints the relative speed values were calculated based on a comparison of the spectrally sensitized materials with the material without spectral sensitizer to which arbitrarily the speed value of 100 was given.

The relative speed values are listed hereinafter.

TABLE V

| No.    | Structural formula of spectral sensitizing agent | Relative speed value |
|--------|--------------------------------------------------|----------------------|
| 0..... | None.....                                        | 100                  |
| 1..... |                                                  | 4,000                |
| 2..... |                                                  | 4,000                |
| 3..... |                                                  | 250                  |
| 4..... |                                                  | 600                  |
| 5..... |                                                  | 1,600                |
| 6..... |                                                  | 250                  |
| 7..... |                                                  | 1,600                |

Table V—Continued

| No.     | Structural formula of spectral sensitizing agent | Relative speed value |
|---------|--------------------------------------------------|----------------------|
| 8.....  |                                                  | 4,000                |
| 9.....  |                                                  | 250                  |
| 10..... |                                                  | 400                  |
| 11..... |                                                  | 400                  |
| 12..... |                                                  | 1,600                |
| 13..... |                                                  | 1,600                |

## EXAMPLE 7

An electrophotographic recording material was prepared by coating onto a conductive layer as described in Example 3 a solution containing :

|                                                                                        |           |
|----------------------------------------------------------------------------------------|-----------|
| Compound 5 of Table II.....                                                            | 3.75 g.   |
| Copoly(vinyl chloride/vinyl acetate/maleic anhydride)-<br>(molar ratio 86.5/13.3/0.2). | 5.0 g.    |
| 1,2-dichloroethane.....                                                                | 70 ml.    |
| Methylene chloride.....                                                                | 20 ml.    |
|                                                                                        | 0.0025 g. |
|                                                                                        | 0.0075 g. |
|                                                                                        | 20        |
|                                                                                        | 0.0280 g. |
|                                                                                        | 30        |
|                                                                                        | 0.0280 g. |
|                                                                                        | 40        |

The coating was carried out at a coverage of 1.35 g of photoconductor per sq.m.

After a negative corona charging the recording layer was exposed in a microfilm camera for 10 sec. with 1,500 lux to a halftone multicolour original. The dia-phragma setting was 4.5 and the original was reduced optically 20 times. The obtained electrostatic charge image was developed as described in Example 1.

We claim:

1. In a recording process wherein a photoconductive insulating recording layer is exposed to an electromagnetic radiation image to produce an imagewise pattern of increased conductivity in said photoconductive recording element and said conductivity pattern is developed to produce a record of said image, the improvement wherein said element comprises an organic photoconductive compound corresponding to the following general formula:



wherein:

$Z_1$  represents the necessary atoms to close an adjacent aromatic nucleus or an adjacent aromatic ring system including such a nucleus or ring system substituted with one or more substituents having a non-ionic character,

5  $R_1$  represents hydrogen, an aliphatic radical, or an alkylene group which is ring closed with the carbon atom in peri-position of the aromatic ring closed by  $Z_1$ , and  $R_2$  represents hydrogen or a lower alkyl group.

2. A recording process according to claim 1, wherein  $R_1$  represents an alkyl radical introduced by alkylation.

3. A recording process according to claim 1, wherein  $Z_1$  represents the necessary atoms to close an adjacent 10 benzene nucleus.

4. A recording process according to claim 1, wherein each  $R_2$  represents a methyl group.

5. A recording to claim 1, wherein the photoconductive compound corresponds to the following general 15 formula:



25 wherein :

$Z_1$  represents the necessary atoms to close an adjacent aromatic nucleus or an adjacent aromatic ring system including such a nucleus or ring system substituted with one or more substituents having a non-ionic character,  $A$  represents an alkylene group, or an alkylene chain interrupted by a bivalent aromatic group, and  $R_2$  represents hydrogen or a lower alkyl group.

30 6. A method for recording and reproducing information comprising the steps of producing an electrostatic charge pattern by electrostatically charging and information-wise exposing to electromagnetic radiation a recording element containing a photoconductive compound corresponding to the following general formula:



35 50 wherein:

$Z_1$  represents the necessary atoms to close an adjacent aromatic nucleus or an adjacent aromatic ring system including such a nucleus or ring system substituted with one or more substituents having a non-ionic character,

$R_1$  represents hydrogen, an aliphatic radical, or an alkylene group which is ring closed with the carbon atom in peri-position of the aromatic ring closed by  $Z_1$ , and

55 60  $R_2$  represents hydrogen or a lower alkyl group, producing thereby an information-wise increase of the conductivity in the recording element, and developing the resulting latent electrostatic charge pattern with a substance that can be electrostatically attracted.

65 7. A process according to claim 1, wherein the recording element is a recording layer that has been applied to an electro conductive layer or support having a resistivity lower than that of the dark-adapted record-

ing element.

8. A process according to claim 7, wherein the electro conductive layer or support has a resistivity at least  $10^2$  as low as that of the recording element in the dark.

9. A process according to claim 7, wherein the support is a paper support.

10. A process according to claim 7, wherein the support is an insulating transparent resin support coated with a transparent electroconductive interlayer.

11. A process according to claim 10, wherein said interlayer contains a polyionic resin.

12. A process according to claim 1, wherein the photoconductive compound is used in admixture with a polymeric binding agent.

13. A process according to claim 1, wherein the photoconductive compound is used in admixture with a halogen-containing polymer, an epoxy resin and/or silicone resin.

14. A process according to claim 13, wherein the halogen-containing polymer contains vinyl chloride units.

15. A process according to claim 1, wherein the photoconductive compound is used in admixture with a substance increasing the photosensitivity of the recording element.

16. A process according to claim 1, wherein the photoconductive compound is used in admixture with a spectral sensitizing dye.

17. A process according to claim 1, wherein the defined organic photoconductive compound is used in admixture with (an) other inorganic and/or organic photoconductive substance(s).

18. A recording material containing a photoconductive insulating recording element capable of being electrostatically charged in the absence of active electromagnetic radiation and capable of retaining the applied charge for a period of time long enough to produce thereon a developed electrostatic charge pattern, characterized in that the recording element stands in electroconductive relationship to a layer or support with a lower resistivity than that of the recording element and in that the recording element contains an organic photoconductive compound corresponding to the following general formula:



wherein :

$Z_1$  represents the necessary atoms to close an adjacent aromatic nucleus or an adjacent aromatic ring system including such a nucleus or ring system substituted with one or more substituents having a non-ionic character,

$R_1$  represents hydrogen, an aliphatic radical or an alkylene group which is ring closed with the carbon atom in peri position of the aromatic ring closed by  $Z_1$ , and

$R_2$  represents hydrogen or a lower alkyl group.

19. A recording material according to claim 18, wherein  $R_1$  represents an alkyl radical introduced by alkylation.

20. A recording material according to claim 18,

wherein  $Z_1$  represents the necessary atoms to close an adjacent benzene nucleus.

21. A recording material according to claim 18, each  $R_2$  represents a methyl group.

22. A recording material according to claim 18, wherein the photoconductive compound corresponds to the following general formula:



wherein :

$Z_1$  represents the necessary atoms to close an adjacent aromatic nucleus or an adjacent aromatic ring system including such a nucleus or ring system substituted with one or more substituents having a non-ionic character,  $A$  represents an alkylene group, or an alkylene chain interrupted by a bivalent aromatic group, and  $R_2$  represents hydrogen or a lower alkyl group.

23. A recording material according to claim 22, wherein  $Z_1$  represents the necessary atoms to close an adjacent benzene nucleus or adjacent benzene nucleus substituted with methyl or alkoxy, and  $A$  represents an alkylene group, a substituted alkylene group or an alkylene chain interrupted by a bivalent aromatic group.

24. A recording material according to claim 18, each  $R_2$  represents a methyl group.

25. A recording material according to claim 18, wherein the recording element is a supported or self-supported layer.

26. A recording material according to claim 18, wherein the recording element contains said organic photoconductive compound in an amount of at least 5 percent by weight.

27. A recording material according to claim 18, wherein the recording element is in layer or sheet form and stands in electroconductive contact with a layer or support that has a resistivity being at least  $10^2$  times as low as that of the recording element in the dark.

28. A recording material according to claim 18, wherein the support is a paper support.

29. A recording material according to claim 18, wherein the support is an insulating transparent resin support coated with a transparent electroconductive interlayer.

30. A recording material according to claim 29, wherein said interlayer contains a polyionic resin.

31. A recording material according to claim 18, wherein the organic photoconductive compound is used in admixture with a polymeric binding agent.

32. A recording material according to claim 31, wherein the photoconductive compound is used in admixture with a halogen-containing polymer, epoxy resin and/or silicone resin.

33. A recording material according to claim 18, wherein the organic photoconductive compound is used in admixture with a spectral sensitizing dye.

34. A recording material according to claim 18, wherein the organic photoconductive compound is used in admixture with (an) other inorganic and/or other organic photoconductive substance(s).

35. A recording material according to claim 34, wherein the organic photoconductive compound is

used in admixture with a photoconductive compound selected from the group of photoconductive selenium and the photoconductive oxides, sulphides and selenides of zinc, cadmium, mercury, antimony, bismuth and lead.

36. A recording material according to claim 18, wherein the photoconductive recording element has an optical density not higher than 0.30 for visible light or copying light.

37. A recording material according to claim 33, wherein the recording element contains a spectrally sensitizing triarylmethane dye, xanthene dye and/or methine dye.

38. A recording material according to claim 18, wherein the recording element contains as chemical sensitizing agent a compound having (a) substituent(s) with strong electron-attracting (electro-negative) character.

39. A recording material according to claim 38, wherein the chemical sensitizing agent is a non-ionic Lewis acid compound.

40. A recording material according to claim 39, 10 wherein the chemical sensitizing agent is a quinone, which is substituted with halogen or cyano.

\* \* \* \* \*

15

20

25

30

35

40

45

50

55

60

65

UNITED STATES PATENT OFFICE  
CERTIFICATE OF CORRECTION

Patent No. 3,798,031 Dated March 19, 1974

Inventor(s) Wilhelmus JANSSENS et al

It is certified that error appears in the above-identified patent and that said Letters Patent are hereby corrected as shown below:

Column 29, Claim 1, lines 50 & 51, change "developed"  
to -- used --.

Signed and sealed this 9th day of July 1974.

(SEAL)  
Attest:

McCoy M. GIBSON, JR.  
Attesting Officer

C. MARSHALL DANN  
Commissioner of Patents